

Patented Jan. 4, 1944

2,338,663

# UNITED STATES PATENT OFFICE

2,338,663

## HYPOL ELIMINATOR SOLUTION

Lowell E. Muehler, Rochester, N. Y., assignor to  
Eastman Kodak Company, Rochester, N. Y., a  
corporation of New Jersey

No Drawing. Original application September 30,  
1941, Serial No. 413,001. Divided and this ap-  
plication September 30, 1941, Serial No. 413,002

6 Claims. (Cl. 95—88)

This invention relates to solutions for use in  
the elimination of hypo from photographic  
images.

This application is a division of U. S. patent  
application Serial No. 413,001, filed September  
30, 1941.

In the processing of photographic developing-  
out materials such as gelatino-silver halide emul-  
sions coated on paper, film, or glass supports, if  
after fixation, the hypo (sodium or ammonium  
thiosulfate) is not completely eliminated from the  
processed material by washing or other means,  
under suitable conditions of temperature and  
humidity during storage, the silver image will  
tend to "fade." This change involves conversion  
of some of the silver to less visible yellowish silver  
sulfide.

When one uses alkaline aqueous solutions con-  
taining compounds which form complex silver  
compounds, such as solutions of ammonia or  
amines; for the purpose of treating fixed paper  
prints, films, and plates to assist in the removal  
of the thiosulfate compounds during the treat-  
ment or in subsequent washing, or to act in con-  
junction with hydrogen peroxide in suitable con-  
centrations for sufficiently oxidizing the thio-  
sulfate to neutral sulfate, it is found that the  
tone of the images, particularly those of fine-  
grain materials such as prints, is altered from a  
warm black to a more bluish-black in the low  
and intermediate densities and to a warmer or  
less dense black in the higher densities. This  
effect while desirable for certain purposes is, by  
virtue of the alteration in tone, sometimes undesir-  
able.

It has been found that this alteration of tone  
can be decreased, and in some cases prevented  
by adding to the ammonia or amine-containing  
solution a soluble compound which is capable of  
forming silver compounds which are insoluble or  
slightly or difficultly soluble in the ammonia or  
amine solution. Suitable compounds in all such  
solutions including those containing hydrogen  
peroxide, are alkali metal halides, such as potas-  
sium bromide and potassium iodide. The halide  
acids, hydrochloric and hydroiodic, and their solu-  
ble ionizable salts with ammonia, organic amines,  
and other organic compounds may also be em-  
ployed in place of the alkali metal bromides and  
iodides. In addition, organic reactants for silver  
are also effective.

The method used for treating prints in the  
manner of my invention includes: washing the  
fixed prints for about 10 to 15 minutes, treating  
with the alkaline peroxide solutions for 5 to 10  
minutes, and washing for 5 to 10 minutes. In  
case alkaline solutions containing no peroxide  
are used, the prints may either be washed or not  
washed prior to treatment, as desired. Treat-  
ment may be from 2 to 10 minutes followed by

sufficient washing, for example, about 30 minutes.  
The degree of elimination of hypo depends both  
upon the time of treatment and the degree of  
washing.

5 The following examples show typical solutions  
which may be used according to my invention,  
however, these examples are intended to be illus-  
trative only, and are not exhaustive of the varia-  
tions and equivalents contemplated by my in-  
vention.

### Example 1

|                                      |       |         |
|--------------------------------------|-------|---------|
| Water                                | cc    | 500     |
| Hydrogen peroxide (3% solu-<br>tion) | cc    | 125-500 |
| 15 Ammonia                           | cc    | 10      |
| Potassium bromide                    | grams | 1-10    |
| Water to make                        | liter | 1       |

The amount of bromide in the above formula  
is not critical, however, the indicated range gives  
satisfactory results. In case it is desired to use  
potassium iodide in place of bromide, about 0.1  
to about 2.0 grams is satisfactory.

The following organic reactions for silver may  
25 be substituted for bromide or iodide in the above  
example:

|                             | Grams   |
|-----------------------------|---------|
| 1,2,3-benzotriazole         | 0.1-1.0 |
| 5-(or 6-)bromobenzotriazole | 0.1-1.0 |
| 30 6-nitrobenzimidazole     | 0.1-0.5 |
| 5-(or 7-) nitroindazole     | 0.1-0.5 |
| 5-aminotetrazole            | 0.1-1.0 |
| 2-aminobenzothiazole        | 0.1-1.0 |
| 2-acetylaminobenzothiazole  | 0.1-0.5 |

35 The organic compounds may be added as alco-  
hol solutions or in the form of their water soluble  
salts. When sufficiently soluble in water such as  
with benzotriazole, they may be added directly.

### Example 2

|                       |       |      |
|-----------------------|-------|------|
| Water                 | liter | 1    |
| Ammonia (28 per cent) | cc    | 5-25 |

45 To this solution may be added any one of the  
following:

|                              | Grams   |
|------------------------------|---------|
| Potassium bromide            | 1-10    |
| Potassium iodide             | 0.1-2   |
| 50 6-nitrobenzimidazole      | 0.1-0.5 |
| 1,2,3-benzotriazole          | 0.1-1.0 |
| 5-(or 6-) bromobenzotriazole | 0.1-1.0 |
| 5-(or 7-) nitroindazole      | 0.1-0.5 |
| 2-mercaptopbenzothiazole     | 0.1-0.5 |
| 55 2-mercaptopbenzoxazole    | 0.1-0.5 |
| 2-aminobenzothiazole         | 0.1-1.0 |
| 5-aminotetrazole             | 0.1-1.0 |
| Thiobenzanilide              | 0.1-0.5 |
| 2-acetylaminobenzothiazole   | 0.1-0.5 |

60 The compounds may be added as noted above.

*Example 3*

The solid chemicals either mixed or unmixed and packaged for later dissolving in a liter of water to make an ammoniacal hypo eliminator bath, may contain 5 to 30 grams of 2-amino-2-methyl-1,3-propandiol and one of the addition substances shown in Example 2, such as 1 to 10 grams of potassium bromide.

The 2-amino-2-methyl-1,3-propandiol compound may be replaced by a similar quantity of a polyalkylene polyamide such as piperazine, di-isopropanolamine, or other solid water soluble alkaline reacting amine or substituted amine the normal solutions of which give a pH value in the range 9.5-12.0.

As another alternative for the solid amine, a water soluble amine salt packaged to be used in conjunction with an inorganic alkali but not necessarily mixed with it may be employed to form a solution. In this manner amines which are not solid at ordinary temperatures may be generated in solution by the addition of alkalies such as sodium carbonate, trisodium phosphate, sodium hydroxide, lithium hydroxide, etc. Ammonium salts such as the chloride and sulfate may also be used in the same manner as the amine salts in conjunction with the inorganic alkalies.

*Example 4*

|                              | Grams |
|------------------------------|-------|
| Diethylamine hydrochloride   | 11    |
| Trisodium phosphate (cryst.) | 38    |

These solid chemicals may be placed in separate compartments of a 2-compartment package. Either compartment may contain 1.0 gram of potassium iodide. The chemicals of the two compartments are for the preparation of one liter of hypo eliminator solution.

*Example 5*

A concentrated solution for marketing to be diluted with water for use in preparing one liter of hypo eliminator solution may contain:

|                  | Grams   |
|------------------|---------|
| Ethanolamine     | 10-20   |
| Hydrobromic acid | 1-5     |
| or               |         |
| Hydriodic acid   | 0.2-1.5 |

The term "ammoniacal" as used herein is not intended to limit the scope of my invention to ammonia or ammonia-peroxide hypo eliminator solutions and refers to the use of ammonia or amines such as ethyl or butyl amine, ethanolamine, diethanolamine, ethylenediamine, diaminopropanol, diethylamine, piperidine, morpholine, cyclohexylamine, benzylamine, triethylamine, and water soluble derivatives which may be either liquids or solids at ordinary temperatures and characterized by the fact that their 0.1

normal solutions give a pH value in the range of 9.5 to 12.0.

One theory of the function of the compounds used in the ammonia solutions appears to be that they prevent solubilizing or changing the surface of the silver images. Thus, sodium chloride is not suitable for use in the solutions of my invention since silver chloride is readily soluble in ammonia. In the ammoniacal peroxide solutions of my invention the compounds appear to precipitate the silver of silver-thiosulfate complexes and delay or prevent both its reduction to silver and the formation of silver sulfide on the image grains. The addition compounds are likewise effective in alkaline and alkaline peroxide hypo eliminator solutions containing no ammonia or amine.

It is to be understood that the disclosure herein is by way of example and that I consider as included in my invention all modifications and equivalents falling within the scope of the appended claims.

## What I claim is:

1. The method of elimination of hypo from photographic silver images which comprises treating said images with an ammoniacal peroxide solution of a heterocyclic nitrogen compound forming a substantially insoluble salt with silver in ammoniacal solution.

2. The method of elimination of hypo from photographic silver images which comprises treating said images with an ammoniacal peroxide solution of 6-nitrobenzimidazole.

3. The solid chemicals packaged for use in making an ammoniacal hypo eliminator bath by dissolving in water for treatment of photographic silver images comprising a solid alkaline reacting water soluble amine and a heterocyclic nitrogen compound forming a substantially insoluble salt with silver in ammoniacal solution.

4. The solid chemicals packaged for use in making an ammoniacal hypo eliminator bath by dissolving in water for treatment of photographic silver images comprising a solid alkaline reacting water soluble amine and a derivative of benzothiazole.

5. The method of elimination of hypo from photographic silver images which comprises treating said images with an ammoniacal solution of a heterocyclic nitrogen compound forming a substantially insoluble salt with silver in ammoniacal solution.

6. The packaged chemicals for use in making an ammoniacal hypo elimination bath by the addition of water for treatment of photographic silver images comprising an alkaline reacting water soluble amine and a heterocyclic nitrogen compound forming a substantially insoluble salt with silver in ammoniacal solution.

LOWELL E. MUEHLER.

CERTIFICATE OF CORRECTION.

Patent No. 2,338,663.

January 4, 1944.

LOWELL E. MUEHLER.

It is hereby certified that error appears in the printed specification of the above numbered patent requiring correction as follows: Page 1, second column, line 24, Example 1, for "reactions" read --reactants--; page 2, first column, line 12, Example 3, for "polyamide" read --polyamine--; and that the said Letters Patent should be read with this correction therein that the same may conform to the record of the case in the Patent Office.

Signed and sealed this 29th day of February, A. D. 1944.

Leslie Frazer

(Seal)

Acting Commissioner of Patents.